

## UNITED STATES PATENT OFFICE

FREDERICK F. MCINTOSH, OF GLEN OSBORNE, PENNSYLVANIA, ASSIGNOR TO CRUCIBLE STEEL COMPANY OF AMERICA, A CORPORATION OF NEW JERSEY

## MANUFACTURE OF STEEL

No Drawing.

Application filed May 6, 1929. Serial No. 361,011.

In an application for Letters Patent filed by me on May 4, 1929, Serial No. 360,613, I have described and claimed a new composition of steel characterized by high content of sulphur, together with a content of molybdenum. In the manufacture of this steel I have also invented a new method of manufacture, which is the invention to which this application is directed.

10 In the manufacture of the steel referred to, I obtain the desired high sulphur content, together with the molybdenum content, by adding to the refined steel while it is still in a molten condition the required quantity 15 of the natural ore of molybdenum, known as molybdenite. In its purity the chemical formula of molybdenite is  $MoS_2$ , and it contains about 40% of sulphur and about 60% of molybdenum. This molybdenum sulphide 20 is added to the refined molten steel either in the ladle or as it is poured into the mold.

Heretofore it has been the general practice in the manufacture of steel containing molybdenum, to add the molybdenum to the furnace charge or to the molten steel in the melting-furnace. The molybdenum is usually added in the form of a so-called calcium molybdate or a ferro molybdate. The reason for adding the molybdenum composition to the steel in the melting-furnace is that 30 it is difficult to get an even distribution of the molybdenum throughout the molten mass of the steel, for it is the fact that molybdenum is rather slow to alloy with the steel. In adding molybdenite to the molten steel in the 35 ladle or in the ingot mold, I have found that I obtain a rapid alloying action of both elements of the addition, and an even diffusion of the elements throughout the mass, without in any way impairing the quality of the 40 steel. The molybdenum sulphide combines readily with the molten steel, and practically none of either component is lost; so that in practice it has been found that when the 45 molybdenum sulphide is added to the molten steel in this way, it will yield about 1.5 points of molybdenum to each point of sulphur added. In this way the sulphur content of the steel is increased to the required amount, 50 and the very valuable element molybdenum

is added at the same time at a very small cost.

The steel may be melted and refined in any suitable melting and refining furnace, either a Bessemer converter, an open-hearth furnace, or an electrical furnace, it being only 55 essential that the steel shall be withdrawn from the refining furnace and that the molybdenite shall be added to the steel while the latter is still in molten condition.

I claim as my invention:

60 The method of manufacture of steel which comprises melting and refining the steel, withdrawing the product from the refining furnace, and while it is still molten adding to it a predetermined quantity of molybdenum sulphide. 65

In testimony whereof I have hereunto set my hand.

FREDERICK F. MCINTOSH.

70

75

80

85

90

95

100